

# United States Patent Office

3,010,900

Patented Nov. 28, 1961

1

## 3,010,900 OIL COMPOSITIONS CONTAINING ALUMINUM DISOAP AND AN AMINE

Hugh H. Horowitz, Elizabeth, and Eric O. Forster, Scotch  
Plains, N.J., assignors to Esso Research and Engineer-  
ing Company, a corporation of Delaware  
No Drawing. Filed May 19, 1958, Ser. No. 735,932  
7 Claims. (Cl. 252—37)

This invention relates to an additive system for improving the viscosity-temperature characteristics of lubricating oil. Particularly, the invention relates to lubricating oil compositions containing a combination of aluminum soap and an amine for improving the viscosity index (V.I.) of the composition.

Recently there has been a marked growth in the use of multi-grade lubricating oils for automotive lubrication. These oils contain V.I. improving additives which minimize the viscosity change of the oil with temperature thereby permitting the use of the same oil over a wide temperature range. This viscosity change in commercial multi-grade oils is usually regulated by high molecular weight polymers such as polymethacrylates and polyisobutylene. However, these long chain polymers tend to irreversibly break down into smaller chains in actual crankcase use. In fact, the chains are literally sheared by the moving parts of the engine and their effectiveness is permanently decreased upon use. It had been known that aluminum hydroxy disoaps tend to associate together to form long chains, somewhat akin to those of the previously described polymers. However, it had not been possible to make effective use of these long chain aluminum soaps for purposes of regulating the viscosity-temperature relationship of lubricating oil. Thus, these aluminum disoaps form extremely long chains which produce a gelling effect upon the oil, and in large concentrations will actually form solid greases. If an attempt is made to form a fluid lubricant by reducing the concentration of the aluminum disoap in oil, then phase separation occurs and a non-homogeneous system results. It has now been found that by using the aluminum disoap in conjunction with certain amines it is possible to effectively regulate the length of the aluminum disoap chain and to improve substantially its V.I. improving powers. Thus, the gelling effect is inhibited and at the same time the disoap chains will function more like the aforementioned long chain hydrocarbon polymers in regulating the viscosity index of lubricating oils. Not only is no gel formed at lower temperatures but the thickening effect of the amine-disoap system is actually less at low temperatures than at high temperatures.

One important advantage of the aluminum disoap chains is that they do not show any substantial permanent shear breakdown, due to the unique ability of the soap chains to reform themselves if broken. In fact, there may be a continuous equilibrium between the formation and rupture of chain links when the disoap is in oil solution. This unique ability of reformation permits extended use of the oil composition without the loss of viscosity-temperature characteristics. Another advantage of the present additive system is that in addition to the V.I. improving function, both the aluminum disoap and the amines function as oil detergents.

The aluminum hydroxy disoaps operable in this invention are formed from straight or methyl-branched, saturated and unsaturated, unsubstituted monocarboxylic acids which preferably contain about 8 to 12 carbon atoms per molecule, e.g. fatty acids such as octanoic, nonanoic, lauric acid, etc. Chain lengths less than 8 carbon atoms are not too desirable since they result in soaps unduly soluble in the oil, while longer chain lengths result in too great a thickening effect. The amines oper-

2

able for limiting or "blocking" the aluminum disoap chain are those having the general formula:



wherein R is an aliphatic, straight or branched hydrocarbon radical which may be ether interrupted, and contains a total of 1 to 22, preferably 8 to 18, carbon atoms; R' is preferably hydrogen, or a short alkyl group such as a methyl radical, and R'' can be the same as R or R'.

10 The disoap and the amine are used together in ratios such that there is about .01 to 1.0, e.g. .2 to .5 part by weight of the amine per one part by weight of the aluminum disoap. In turn, this additive combination, i.e. disoap and amine, can be used in finished lubricating oils in amounts of 0.5 to 10, e.g. 1.5 to 3.5 weight percent, based on the total weight of the oil composition. For ease of handling, oil concentrates of these additives may 15 also be prepared which may contain 5 to 30 wt. percent additive.

15 The lubricating oils which can be improved in their viscosity index by the above described additive combination will include mineral lubricating oils, synthetic lubricating oils, or mixtures thereof. Synthetic lubricating oils which may be used include esters of dibasic acids (e.g. di-2-ethylhexyl sebacate); esters of glycols (e.g. C<sub>13</sub> Oxo acid diester of tetraethylene glycol); complex esters (e.g. the complex ester formed by reacting one mole 20 of sebacic acid with two moles of tetraethylene glycol and two moles of 2-ethylhexanoic acid); formals; silicones; carbonates; polyglycols and other synthetic lubricating oils known in the art.

25 Although of primary advantage for use in lubricating oils intended for automotive crankcase use, the additive combination of the invention may be used in other oil compositions, such as: turbine oils, industrial oils, oils for atomic installations, hydraulic and transmission fluids, heating oils, etc.

30 35 40 In evaluating the effectiveness of the additive systems of the invention in improving the viscosity-temperature characteristics of lubricating oil two criteria were used. One criteria was the common Dean and Davis Viscosity Index relationship which is fully described in A.S.T.M. 45 D-567. This relationship is as follows:

$$\text{V.I.} = \frac{L-U}{L-H} \times 100$$

45 50 where:

U is the viscosity at 100° F. of the oil under consideration. L is the viscosity at 100° F. of a zero=V.I. oil having the same viscosity at 210° F. as the oil under consideration.

55 H is the viscosity at 100° F. of a 100 V.I. oil having the same viscosity at 210° F. as the oil whose viscosity is being tested.

60 65 In order to apply the above formula, the viscosities of the oil under consideration at 100° F. and 210° F. must be determined, and may be expressed in either centistokes or in Saybolt Universal seconds. Values for L and H are taken from tables.

70 75 Although the Dean and Davis V.I. scale is widely used to express numerically the viscosity-temperature relationship for an oil, it is not too well suited for use in the range of 150 V.I., the range of interest here, because of anomaly in the V.I. system and because the V.I. level is sharply dependent on the viscosity level at which the measurement is made.

75 80 Therefore in an attempt to more effectively evaluate the viscosity-temperature relationships imparted by the

3  
additive systems of the invention, a second relation was used which consisted of the following equation;

$$S = \frac{\eta Sp \text{ } 100^\circ \text{ F.}}{\eta Sp \text{ } 210^\circ \text{ F.}}$$

wherein:

S is a numerical value expressing the rate of change of viscosity with temperature. Thus, the lower the value of S, the less the additive thickens at lower temperature and the better the oil composition in this respect.  $\eta Sp \text{ } 100^\circ \text{ F.}$  is the increase in viscosity in centistokes at  $100^\circ \text{ F.}$  contributed by the additive, divided by the viscosity of the base oil in centistokes at  $100^\circ \text{ F.}$  That is

$$\eta Sp \text{ } 100^\circ \text{ F.} = \frac{\eta_{\text{blend}} - \eta_{\text{base oil}}}{\eta_{\text{base oil}}}$$

$\eta Sp \text{ } 210^\circ \text{ F.}$  is a ratio similar to  $\eta Sp \text{ } 100^\circ \text{ F.}$ , except that the viscosities are obtained at  $210^\circ \text{ F.}$

Of the two numerical measures of the viscosity-temperature relationship discussed above, the S value is a more useful relationship. In the case of polymeric additives it is relatively independent of the viscosity of the base stock and the concentration of the additive. It thus allows for a direct comparison of additives without the confusing effects of viscosity and concentration. In sum, the lower the S value, the more effective the additive functions as a V.I. improver.

The invention will be further understood by the following examples:

#### EXAMPLE I

A series of lubricating oil blends were prepared by simple mixing of an aluminum hydroxy di-n-octanoate and various amine blocking agents in a solvent extracted mineral lubricating oil containing bright stock. The amines used were: lauryl dimethyl amine, n-octyl amine, Primene JMT (Rohm and Haas) which is a tertiary alkyl primary amine having predominantly 18 carbon atoms per molecule with minor amounts of homologous molecules of 19 to 24 carbon atoms, Amine 9D-178 (Rohm and Haas) which is a mixture of highly branched unsaturated secondary aliphatic amines having an average molecular weight of 375, and Alkyl Ether Amine #1 (Archer-Daniels-Midland), which has the formula:



wherein R represents about a 50/50 mixture of alkyl groups containing 14 and 16 carbon atoms each, derived from commercial lauric acid.

The exact compositions prepared and their viscosity-temperature relationship are given in Table I which follows:

Table I

BLEND'S OF Al DIOCTANOATE AND VARIOUS AMINES IN MINERAL LUBRICATING OIL

| Composition | Alumi-<br>num di-<br>octanoate<br>weight<br>percent | Weight percent blocking agent         | Vis./<br>210° F.<br>cp. | Vis./<br>100° F.<br>cp. | $\eta Sp$<br>210° F. | $\eta Sp$<br>100° F. | $S =$<br>$\eta Sp \text{ } 100^\circ \text{ F.}$<br>$\eta Sp \text{ } 210^\circ \text{ F.}$ | V.I.<br>(Dean<br>and<br>Davis) | Gelling<br>effect<br>at $77^\circ \text{ F.}$ |
|-------------|-----------------------------------------------------|---------------------------------------|-------------------------|-------------------------|----------------------|----------------------|---------------------------------------------------------------------------------------------|--------------------------------|-----------------------------------------------|
| A.          | 0.0                                                 | 0.0                                   | 9.51                    | 79.96                   | 0.741                | .449                 | .606                                                                                        | 107                            | None.                                         |
| A.          | 1.0                                                 | 0.0                                   | 16.88                   | 115.9                   | .757                 | .332                 | .439                                                                                        | 140                            | Yes.                                          |
| B.          | 1.0                                                 | 0.4 lauryl dimethyl amine             | 16.70                   | 106.7                   | 1.072                | .542                 | .542                                                                                        | 140                            | None.                                         |
| C.          | 1.0                                                 | 0.4 n-octyl amine                     | 28.35                   | 166.3                   | 1.980                | 1.258                | .843                                                                                        | 136                            | Slight.                                       |
| D.          | 1.0                                                 | 0.4 primene JMT 1                     | 25.6                    | 180.7                   | 1.498                | .879                 | .792                                                                                        | 133                            | Do.                                           |
| E.          | 1.0                                                 | 0.4 Amine 9D-178 <sup>2</sup>         | 20.05                   | 150.2                   | 1.11                 | .0305                | .0086                                                                                       | 111                            | Do.                                           |
| F.          | 1.0                                                 | 0.4 alkyl ether amine #1 <sup>1</sup> | 9.88                    | 80.65                   | 2.61                 | 2.064                | .280                                                                                        | 141                            | None.                                         |
| G.          | 2.0                                                 | 0.0                                   | 34.30                   | 245.4                   | 1.275                | .429                 | .792                                                                                        | 135                            | Yes.                                          |
| H.          | 2.0                                                 | 0.4 lauryl dimethyl amine             | 37.74                   | 181.9                   | 2.97                 | 1.275                | .429                                                                                        | 142                            | None.                                         |
| I.          | 2.0                                                 | 0.4 alkyl ether amine #1              | 13.70                   | 98.6                    | .442                 | .233                 | .528                                                                                        | 131                            | Do.                                           |

<sup>1</sup> Mixture of  $C_{18-24}$  tertiary alkyl primary amines.

<sup>2</sup> Mixture of highly branched-chain secondary aliphatic amines, average molecular weight of 375.

<sup>3</sup>  $\text{ROCH}_2\text{CH}_2\text{CH}_2\text{NH}_2$  where R represents alkyl radicals derived from commercial lauric acid.

As seen from the preceding table, the base oil had an initial V.I. (Dean and Davis) of 107. The addition of 1 wt. percent of aluminum dioctanoate (A) resulted in an S value of 0.606 and a V.I. of 140. However, at  $77^\circ \text{ F.}$  this composition formed a gel, i.e. a grease-like material, due to the unregulated thickening effect of the aluminum disoap. The addition of the lauryl dimethyl amine (B) eliminated the gelling effect of the disoap, while further lowering the S value. The n-octyl amine (C), the Primene JMT (D) and Amine 9D-178 (E) were also effective with the aluminum disoap, although they did show a slight gelling effect at  $77^\circ \text{ F.}$  This slight gelling effect was not too serious since it can be removed and a homogeneous product formed by milling the composition, e.g. by passing the composition through a Morehouse mill or a Gaulin homogenizer.

The alkyl ether amine #1 (F) was quite effective, showing no gelling tendency and a very low S value, although it should be noted that this value is not too precise, being the ratio of two small numbers. Compositions G, H and I illustrate the use of larger amounts of the disoap, and here again it is seen that the lauryl dimethyl amine and the alkyl ether amine #1 were both quite effective in preventing gelling while at the same time maintaining a good viscosity-temperature relationship.

#### EXAMPLE II

A second series of lubricating oil compositions were prepared by simple mixing of varying amounts of an aluminum hydroxy di-n-decanoate and alkyl ether amine #1, in a neutral paraffinic mineral oil having a viscosity of 150 SUS. at  $100^\circ \text{ F.}$  The compositions prepared and their viscosity-temperature characteristics are summarized in Table II which follows:

Table II

VISCOSITY-TEMPERATURE CHARACTERISTICS OF BLENDS OF ALUMINUM DIDEcanoATE AND ALKYL ETHER AMINE #1 IN OIL

| Al soap<br>conc.,<br>weight<br>percent | Alkyl<br>ether<br>amine #1<br>weight<br>percent | Vis./20<br>(cs.) | Vis./100<br>(cs.) | Vis./210<br>(cs.) | $S =$<br>$\eta Sp \text{ } 100^\circ \text{ F.}$<br>$\eta Sp \text{ } 210^\circ \text{ F.}$ | V.I.  |
|----------------------------------------|-------------------------------------------------|------------------|-------------------|-------------------|---------------------------------------------------------------------------------------------|-------|
| 0                                      | 0                                               | 458.2            | 31.74             | 5.30              | -----                                                                                       | 110   |
| 0.5                                    | 0.1                                             | 519.4            | 35.82             | 6.60              | 0.895                                                                                       | 141   |
|                                        | 0.2                                             | 469.9            | 32.10             | 5.36              | -----                                                                                       | 111.5 |
|                                        | 0.4                                             | 462.5            | 31.50             | 5.26              | -----                                                                                       | 110   |
| 1.0                                    | 0.2                                             | 548.6            | 44.79             | 9.01              | 0.587                                                                                       | 154   |
|                                        | 0.3                                             | 496.3            | 38.46             | 7.36              | 0.549                                                                                       | 147   |
|                                        | 0.4                                             | 489.5            | 33.39             | 6.02              | 0.385                                                                                       | 134   |
|                                        | 0.8                                             | 468.0            | 31.95             | 5.39              | -----                                                                                       | 114   |
| 1.5                                    | 0.4                                             | 710.0            | 52.11             | 11.76             | 0.527                                                                                       | 159.5 |
|                                        | 0.6                                             | 573.1            | 37.92             | 7.62              | 0.445                                                                                       | 152.2 |
|                                        | 0.8                                             | 472.6            | 32.31             | 5.60              | 0.315                                                                                       | 123   |
| 2.0                                    | 0.8                                             | 632.0            | 42.24             | 9.98              | 0.380                                                                                       | 164   |

<sup>1</sup>  $\text{ROCH}_2\text{CH}_2\text{CH}_2\text{NH}_2$  where R represents alkyl radicals derived from commercial lauric acid.

As seen from Table II, better and better S values were obtained as the concentration of aluminum disoap and amine blocking agents were increased. The S values below 0.6 are superior to those obtainable with the best commercial V.I. improver. The aluminum disoap alone in the oil and without the amine would have resulted in solid gels at 20° F., even at a concentration of 0.5 wt. percent disoap. However, with the blocking agent present the viscosity of the blend is only slightly higher than the base oil at 20° F.

### EXAMPLE III

A third series of compositions were prepared by simple mixing of aluminum hydroxy di-n-decanoate and lauryl dimethyl amine in varying amounts in a solvent extracted mineral oil containing bright stock. The compositions tested and their properties are summarized in Table III.

Table III

ALUMINUM DIDECAANOATE AND LAURYL DIMETHYL AMINE IN MINERAL OIL

| Alumi-num disoap (weight percent) | Lauryl dimethyl amine (weight percent) | Vis./ 20° F. (cs.) | Vis./ 100° F. (cs.) | Vis./ 210° F. (cs.) | $S = \frac{\eta_{Sp} 100}{\eta_{Sp} 210}$ | V.I. (Dean and Davis) |
|-----------------------------------|----------------------------------------|--------------------|---------------------|---------------------|-------------------------------------------|-----------------------|
| 0.0                               | 0.0                                    | ---                | 111.8               | 11.92               | 0.616                                     | 104.5                 |
| 0.5                               | 0.2                                    | 4.450              | 128.8               | 14.79               | 0.616                                     | 118.5                 |
| 0.6                               | 4.380                                  | 115.9              | 13.86               | 0.188               | 120                                       |                       |
| 1.0                               | 0.2                                    | 5.710              | 185.6               | 30.62               | 0.422                                     | 140                   |
| 1.0                               | 0.4                                    | 5.310              | 153.0               | 21.96               | 0.445                                     | 137                   |
| 1.5                               | 0.1                                    | ∞                  | 372.80              | 74.50               | 0.413                                     | 134                   |
| 1.5                               | 0.6                                    | ∞                  | 275.10              | 47.94               | 0.443                                     | 137                   |

### EXAMPLE IV

A series of oil compositions were prepared by mixing an aluminum disoap prepared from the saturated C<sub>8</sub>-C<sub>12</sub> fraction of cocoanut fatty acids and either lauryl dimethyl amine or alkyl ether amine #1 in a neutral paraffinic mineral lubricating oil. The compositions prepared and their viscosity-temperature characteristics are summarized in Table IV which follows:

Table IV

ALUMINUM DISOAP PREPARED FROM COCOANUT FATTY ACID<sup>1</sup> AND AMINES IN MINERAL LUBRICATING OIL

|                       | Al. disoap, weight percent | Amine, weight percent | Vis./ 20° F. (cs.) | Vis./ 100° F. (cs.) | Vis./ 210° F. (cs.) | $S = \frac{\eta_{Sp} 100}{\eta_{Sp} 210}$ | V.I.  |
|-----------------------|----------------------------|-----------------------|--------------------|---------------------|---------------------|-------------------------------------------|-------|
| Base oil              | 0                          | 0                     | 453.2              | 31.74               | 5.30                | ---                                       | 110   |
| Lauryl dimethyl amine | 1.0                        | 0.2                   | 498.5              | 43.60               | 8.80                | 0.567                                     | 154   |
| Alkyl ether amine #1  | 1.0                        | 0.2                   | 548.6              | 44.79               | 9.01                | 0.587                                     | 154   |
| Lauryl dimethyl amine | 1.5                        | 0.4                   | 490.4              | 127.30              | 22.65               | 0.920                                     | 144.5 |
| Alkyl ether amine #1  | 1.5                        | 0.4                   | 710.0              | 52.11               | 11.76               | 0.527                                     | 159   |

<sup>1</sup> The cocoanut fatty acid consisted of a mixture of about 28 weight percent caprylic, 56 weight percent capric and 16 weight percent lauric acids.

### EXAMPLE V

A composition was prepared consisting of 98.1 wt. percent mineral lubricating oil of 170 SUS. at 100° F., 1.5 wt. percent of aluminum hydroxy disoap of cocoanut fatty acid, (same as in Example IV) and 0.4 wt. percent of alkyl ether amine #1. This composition was tested in actual lubricating use in a laboratory Chevrolet engine. This test involved a 6-cylinder engine running under moderate constant speed and load conditions for 24 hours. The engine stood for another 24 hours before the oil was drained and dismantling began. Oil samples were removed at frequent intervals to follow the change in viscosity. At the end of the test, the engine appeared very clean and no gelling of the oil had occurred.

In summary, this invention relates to an additive combination of an aluminum disoap and certain amines. This combination is extremely effective in improving the

60

65

70

75

80

85

90

95

100

viscosity-temperature characteristics of lubricating oil compositions.

What is claimed is:

- 5 1. A liquid lubricating oil composition comprising a major proportion of a lubricating oil and about 0.5 to 10.0 wt. percent of an additive combination of aluminum hydroxy disoap of a C<sub>8</sub> to C<sub>12</sub> fatty acid and about 0.01 to 1.0 part by weight of an amine per part by weight of said aluminum disoap, wherein said amine 10 has the general formula:



15 wherein R contains a total of about 1 to 22 carbon atoms and is selected from the group consisting of alkyl radicals and ether interrupted alkyl radicals, R' is selected from the group consisting of hydrogen and methyl 20 radicals and R'' is selected from the group consisting of R and R' and wherein said aluminum hydroxy disoap is the sole aluminum soap.

25 2. The liquid lubricating oil composition of claim 1, wherein R', and R'' both represent hydrogen and R represents an alkyl radical.

3. The liquid lubricating oil composition of claim 1, 1, wherein R' and R'' both represent hydrogen and R represents an ether interrupted alkyl radical.

4. The liquid lubricating composition of claim 1, 20 wherein said lubricating oil is a mineral oil.

30 5. The liquid lubricating oil composition of claim 1, wherein said fatty acid is a C<sub>8</sub> fatty acid.

35 6. A method of lubricating an automotive piston engine which comprises operating said engine with the composition of claim 1 in the crankcase of said engine.

7. A liquid lubricating oil composition comprising a major proportion of a mineral lubricating oil and about 1.5 to 3.5 wt. percent of a combination of an aluminum hydroxy disoap of a C<sub>8</sub> to C<sub>12</sub> fatty acid and about 0.2 to 0.5 parts by weight of an amine per part by weight

of said aluminum disoap, wherein said amine has the

general formula:



wherein R contains 8 to 18 carbon atoms and is selected from the group consisting of alkyl radicals and ether interrupted alkyl radicals and R' and R'' represent hydrogen.

References Cited in the file of this patent

#### UNITED STATES PATENTS

- 2,320,002 Lutz et al. May 25, 1943  
 2,491,641 Bondi Dec. 20, 1949  
 2,758,086 Stuart et al. Aug. 7, 1956

#### FOREIGN PATENTS

- 563,429 Great Britain Aug. 15, 1944